

## UNITED STATES PATENT OFFICE.

ANDREW J. CAVANAUGH, JR., OF RICHMOND, VIRGINIA, ASSIGNOR TO THE RANDOLPH PAPER BOX COMPANY, OF RICHMOND, VIRGINIA, A CORPORATION OF VIRGINIA.

## COMPOSITION FOR RENDERING CARDBOARD IMPERVIOUS TO GREASE.

1,357,844.

Specification of Letters Patent.

Patented Nov. 2, 1920.

No Drawing.

Application filed January 5, 1918. Serial No. 210,459.

To all whom it may concern:

Be it known that I, ANDREW J. CAVANAUGH, Jr., a citizen of the United States, residing at Richmond, in the county of 5 Henrico and State of Virginia, have invented certain new and useful Improvements in Composition for Rendering Cardboard Impervious to Grease; and I do hereby declare the following to be a full, 10 clear, and exact description of the invention, such as will enable others skilled in the art to which it appertains to make and use the same.

This invention relates to paper and particularly 15 relates to a composition for application to paper or fibrous material whereby it is rendered substantially impervious to grease, oils, and the like and especially has for its object the preparation of a paste or 20 semiplastic material which may be brushed on to the surface of the paper or fibrous material of whatever its nature which it is desired to treat so as to render it impervious to grease, it being understood that the paste 25 may be applied in any suitable manner as well as by brushing to the surface of the paper, etc., either before or after the paper is shaped into any article of manufacture.

And the invention consists in a combination 30 of ingredients as more particularly set forth hereinafter, and also consists in the method of compounding the paste.

A practical and efficacious composition of the desired nature may be readily made by 35 the mixture of suitable proportions of sodium silicate, mica, glycerin, and powdered dextrin, and in some instances, if preferred there may be added prepared chalk, which latter is utilized to thicken the paste. 40 to bring it to the desired consistency although this may be eliminated when the paste or cement is preferred to be in a thinner or liquid form. It is one of the objects of the present invention to provide a paste 45 of this character which may be made inexpensively and produce the desired properties and characteristics, with the combination of the least possible different ingredients and in the practice of the method of making the 50 paste, a suitable quantity of sodium silicate, say eleven pounds is mixed with about a quarter of a pound of mica and ten ounces

of glycerin, these ingredients being well commingled in any suitable manner and apparatus. To this mixture there may then 55 be added a suitable preparation, for instance, about three ounces of powdered dextrin, which has the property of acting as an adhesive to render a composition more or less densely consistent and also facilitates 60 the drying of the paste.

The several ingredients are preferably mixed in the presence of heated water to facilitate the thorough intermixture of the components, and is then ready to be used by 65 the application by the brush or other method, to the surface of the paper or other fibrous body which it is desired to render impervious to grease.

For the purpose of increasing the thickness or consistency of the preparation, there may be added a quantity of prepared chalk in the proportion of two ounces to the quantities above given for the other ingredients, it being understood however that the proper 75 consistency of the paste may be arrived at by relative variation of the other ingredients, and in their mixture with a greater or larger quantity of water. From the above it will be seen that I have provided a composition of this character, formed of ingredients, all of which are relatively inexpensive, and which form a composition capable of giving to the paper or other fibrous material to be coated, the desired characteristic of being substantially impervious to 80 grease. 85

What is claimed is:

1. A paste for application to paper or other fibrous material, whereby it is rendered impervious to grease, and consisting of a mixture of sodium silicate, mica, powdered dextrin, glycerin and a thickener. 90

2. A material for rendering paper or other fibrous material substantially grease 95 proof, which consists of a mixture in paste form, consisting of eleven pounds of sodium silicate,  $\frac{1}{4}$  of a pound of mica, ten ounces of glycerin, and three ounces of powdered dextrin, and prepared chalk in a sufficient quantity to thicken the material. 100

In testimony whereof I affix my signature.

ANDREW J. CAVANAUGH, Jr.

Sod. Silicate - 176 ozs - 90%

mica - 4 " -

glycerine - 10 " -

water

D - glycerin  
D - Dextrin  
D - Mica